

May 23, 1944.

E. R. BOLLER ET AL

2,349,698

FIBERBOARD

Filed July 1, 1941



*Ernest R. Boller*  
*Raymond F. Remler* INVENTORS

BY

*Albert B. Briggs*  
ATTORNEY

## UNITED STATES PATENT OFFICE

2,349,698

## FIBERBOARD

Ernest R. Boller, Hudson, and Raymond F. Remier, Lakewood, Ohio, assignors to E. I. du Pont de Nemours & Company, Wilmington, Del., a corporation of Delaware

Application July 1, 1941, Serial No. 400,700

2 Claims. (Cl. 154—33.05)

This invention relates to fiberboard and processes for producing it, and is more particularly directed to corrugated fiberboard comprising a paperboard corrugated member impregnated on at least one side with sodium silicate, the ratio between the percentage of sodium silicate on the outside .002 inch of the paper board and in the next lower .002 inch being from about 1.2 to 3.0, and one or more paper linerboards which optionally may be treated with sodium silicate in the same manner as the corrugating medium, and is further directed to processes for producing such fiberboard.

Recently an increasing amount of attention has been devoted to the strength characteristics of corrugated fiberboard shipping containers. There is a growing realization that damages in transit and in storage to goods packaged in such containers can be greatly reduced by observing certain minimum strength standards for the containers, and that these standards can be directly related to the conditions of use. These standards require that the containers be able to stand up under compression tests and other such tests made on the finished containers, on the corrugated fiberboard from which the container is made, and on the materials from which the fiberboard is made.

Fiberboard container manufacturers have endeavored to meet the strength requirements for their products in two ways, first by improving and controlling their operations for producing corrugated fiberboard and for fabricating it into containers, and second by raising the quality and strength properties of the paperboard used in manufacturing the fiberboard containers. Both of these lines of attack must be followed to produce the highest quality of product. Unfortunately, the use of high quality, high strength paperboard has heretofore entailed higher cost, since to obtain such paperboard it has been necessary to use either more fibers or higher quality fibers. This higher cost is probably the chief factor militating against greater and more general improvement in the strength properties of fiberboard containers.

Other methods of adding strength and stiffness to paperboard have been suggested, such as treatment with sodium silicate, and such methods have found a limited usefulness as for instance in coating butter boxes and similar containers, but brittleness caused by such treatment makes the treated paper inapplicable for use as a corrugating medium in corrugated fiberboard. The sharp bending to which a corrugating me-

dium is subjected by the corrugating rolls in the manufacture of fiberboard makes it imperative that brittleness be absent and processes heretofore known for coating paper with sodium silicate have not been free from this troublesome property.

It is an object of this invention to provide improved corrugated fiberboard suitable for use in making containers. Another object is to provide a high quality of corrugated fiberboard assembled from paper of a quality heretofore considered inferior. Another object is to provide fiberboard which for a given strength employs a minimum amount of fiber stock. Another object is to provide processes for producing such improved fiberboard without interference with accepted assembling techniques and machinery. Other objects will appear hereinafter.

The foregoing and other objects of this invention are accomplished by treating a paperboard on at least one side with a sodium silicate solution of such a concentration and  $\text{SiO}_2:\text{Na}_2\text{O}$  weight ratio that with the paperboard used an impregnation of decreasing concentration from outside to inside of the paperboard is obtained, the ratio between the percentage of sodium silicate in the outside .002 inch and in the next lower .002 inch of the side treated being from about 1.2 to 3.0, and assembling the impregnated paperboard into a laminated board. In a preferred embodiment of this invention the impregnation is accomplished in the course of manufacture of the paper by applying a sodium silicate solution at a point between the end of the driers and the end of the calender rolls, the concentration and  $\text{SiO}_2:\text{Na}_2\text{O}$  weight ratio of the silicate solution used being so related to the porosity, moisture content, and fiber character of the paperboard at the point of application that penetration of the silicate into the paper occurs to the extent necessary to give the desired concentration gradient.

In the drawing there is illustrated one particular embodiment of this invention in which a laminated fiberboard is made up of two paperboard plies joined with an adhesive film. In this embodiment the lower paperboard ply has been treated on its lower side with a graduated silicate impregnant, indicated by the dotted portion, the greater density of dots near the lower edge of the bottom paperboard indicating the greater concentration of sodium silicate in that portion of the paperboard and the variation of density of dots being illustrative of the fact that the percentage of sodium silicate in the bottom .002 inch of the paperboard and in the next .002 inch is

from about 1.2 to 3.0. It will be understood that the drawing illustrates but a single embodiment of the invention, and that any desired number of plies might be used, that one or more of the plies might be corrugated, and that some or all of the plies might be impregnated on both sides or on a single side with the graduated silicate impregnant.

Paperboard impregnated with sodium silicate according to a process of this invention has considerably improved properties for use in laminated board, particularly corrugated board and spiral or convolute-wound fiberboard tubes. The treated paperboard has improved stiffness without being brittle. Hence it may be used as a corrugating medium in corrugated board without cracking on the corrugating rolls. Moreover, the corrugated board made with such silicate-treated paperboard has greatly improved strength properties and is of a character ideally adapted for the manufacture of containers.

The nature of this invention and its manner of application will be better understood by reference to the following example which is not to be construed as limited.

#### EXAMPLE

Strawboard .010 inch in thickness and with a basic weight of 35 lbs. per 1000 sq. ft. was treated with sodium silicate solution having a specific gravity of 20° Bé. and a  $\text{SiO}_2:\text{Na}_2\text{O}$  weight ratio of 3.25. The silicate was applied from water boxes on the calender stack of a paper making machine. The equivalent of 4.5 lbs. of 40° Bé. solution was applied per 1000 sq. ft. of strawboard. Application of the silicate in this manner did not necessitate any reduction of speed or other changes in the normal operation on the paper making machine.

The silicate-treated strawboard had a ratio of silicate in the outside .002 inch to that in the next lower .002 inch of 1.48 and a ratio of silicate in the second .002 inch to that in the the third .002 inch of 2.04. The treated strawboard had a crushing strength of 36.0 lbs. in the machine direction and 22.3 lbs. in the cross direction, whereas the untreated strawboard had a crushing strength of 25.8 lbs. in the machine direction and 16.4 lbs. in the cross direction. The strength increase by reason of the silicate treatment, therefore, was 39 per cent in the machine direction and 36 per cent in the cross direction.

The silicate-treated strawboard was used as the corrugating material in fabricating corrugated board, "A" flute, on a conventional pressure-type corrugating machine with 16 point jute linerboard on both the single and double face sides. Sodium silicate was used as the corrugating adhesive. No deviation from the customary corrugating practice was necessary in fabricating this board from the silicate-treated strawboard. Similarly corrugated board was fabricated from the untreated control strawboard under the same conditions. Flatwise crush tests were conducted on specimens of these two boards. The strength of the board constructed with the untreated strawboard was 23.3 lbs./sq. in. and that of the board fabricated from the silicate-treated strawboard was 28.3 lbs./sq. in., the silicate treatment of the corrugating medium accounting for a 21 per cent increase in crushing strength.

The improved character of the fiberboard made with silicate-treated corrugating medium of the example was further demonstrated by

manufacturing boxes from the corrugated board, boxes also being made from the fiberboard having untreated corrugating medium for comparison. These boxes were No. 2 can case size. No differences in behavior of the two boards in this fabricating operation were noted. The boxes were tested in compression, both end to end and top to bottom, ten specimens being tested in each direction. The boxes were set up, all flaps glued, and then conditioned to 7.2 per cent moisture content before testing. The compression strength of the boxes fabricated from the untreated strawboard was found to be 773 lbs. end to end and 793 lbs. top to bottom. The compression strength of the boxes constructed from the silicate-treated strawboard was found to be 997 lbs. end to end and 970 lbs. top to bottom, representing an advantage of 28 per cent and 23 per cent respectively for the latter boxes.

While in the foregoing example certain materials and conditions were employed, it will be understood that the advantages of the invention may be secured with other materials and under other conditions.

To obtain a gradient of sodium silicate concentration in paperboard treated according to a process of this invention, the concentration and  $\text{SiO}_2:\text{Na}_2\text{O}$  weight ratio should be correlated with the properties of the paperboard at the point of application. The factors requiring correlation are enumerated below.

#### 1. Concentration of silicate solution

The concentration of silicate solution applied may be considerably varied, the particular concentration used in a specific instance depending upon the condition of the paperboard at the point of application. The concentration may be such that the silicate solution has a specific gravity in the range of from about 10 to 30° Bé., a gravity of about 20° Bé. being in most instances preferable.

#### 2. $\text{SiO}_2:\text{Na}_2\text{O}$ ratio of silicate

The  $\text{SiO}_2:\text{Na}_2\text{O}$  weight ratio of the silicate used should be from about 3.00 to 3.50 and preferably in the range from 3.00 to 3.30. With ratios above 3.50 the treated paper has a tendency to be brittle and with ratios below 3.00 the alkali tends to strike thru the paper and also the treated paper is slow-drying. Furthermore, treated paperboard made with silicates having ratios outside the ratio range indicated has inferior crushing strength.

#### 3. Porosity of paperboard

The porosity of paperboard treated is an important factor governing the concentration of silicate solution to be used. Ordinarily the porosity of the paperboard depends on the fibers from which the board is made and the extent to which the board has been compacted, as by heavy calendering. Such paperboards as kraft, straw, jute, and chipboard vary considerably in the rates at which they are penetrated by silicate solutions. Chipboard, for instance, being relatively dense and non-porous, requires the use of a relatively dilute silicate solution, say 15 to 20° Bé. or less, in order that the desired concentration gradient from outside to inside may be attained. On the other hand, strawboard, being relatively porous, takes up the silicate solution rapidly and a more concentrated solution, say 20 to 25° Bé. or even higher, proves more satisfactory under ordinary conditions.

#### 4. Moisture content of paper

The moisture content of the paperboard at the point of application of the silicate solution has a considerable influence on the distribution of the silicate to the paperboard. This moisture content may vary considerably, preferably being about 6 to 8 per cent where the paper leaves the driers and where it leaves the calender rolls, and being higher than this at various intermediate points because of water applied from water boxes on the calender rolls. At the lower moisture contents relatively dilute silicate solutions may be applied whereas with higher moisture contents in the paper a more concentrated silicate solution should be used.

#### 5. Size in paper

Other conditions being equal, the amount of size in paperboard treated with a silicate solution influences the distribution of the silicate thru the paperboard. For paperboards containing considerable amounts of size such as kraft it is ordinarily necessary to use a relatively dilute silicate solution, say 10 to 20° Bé., although more concentrated solutions can be used when a wetting agent is employed in the solution to facilitate penetration. With unsized paperboard, on the other hand, a more concentrated solution, say 20 to 30° Bé., should be employed, else the distribution of the silicate in the paper is not graduated but rather, is uniform.

#### 6. Amount of silicate solution applied

The total amount of sodium silicate which is applied to paperboard according to a process of this invention may be varied over a considerable range. Generally it is preferable to use, per thousand square feet of paperboard, an amount of sodium silicate equivalent to from about 1 to 5 lbs. of 40° Bé. solution, lesser amounts giving insufficient strength increase of the paperboard and in some instances being inadequate to establish the desired gradient of silicate content in the paperboard, and larger amounts being generally superfluous and tending to superimpose a surface coating on the paperboard.

#### 7. Thickness of paper

The thickness of a paperboard treated with silicate according to this invention should be in excess of .004 inch for paper coated only on one side and in excess of .006 inch for paper coated on both sides. Ordinarily the paperboard used as corrugating medium will be considerably thicker than this, but it is noted that for corrugated board of equal strength one may start with a lighter weight corrugating medium if a silicate

treatment is to be applied. Thus a strawboard corrugating medium weighing 32 lbs. per 1000 square feet, when treated with sodium silicate, has a strength equivalent to a strawboard weighing 34 lbs. per 1000 square feet. This represents a substantial saving to the paperboard manufacturer since the saving of fiber thus made possible more than offsets the cost of the treatment.

While in the foregoing description of this invention there have been shown numerous processes and products, it will be understood that without departing from the spirit of this invention those skilled in the art may employ various processes for treating paper with sodium silicate and produce numerous treated products.

#### 15. We claim:

1. In a process for producing laminated fiberboard, the steps comprising treating at least one side of a paperboard, which is at least .004 inch thick, with a sodium silicate solution having a specific gravity of from about 10 to 30° Baumé and an  $\text{SiO}_2:\text{Na}_2\text{O}$  weight ratio of from about 3.00 to 3.50, controlling the distribution of the silicate in the paperboard so that the ratio between the percentage of sodium silicate in the outside .002 inch and the next lower .002 inch is from about 1.2 to 3.0, such control being accomplished by varying the silicate solution concentration inversely with the amount of size and directly with the moisture content and porosity of the paperboard, and the total amount of silicate solution applied being equivalent to from about 1 to 5 pounds of 40° Baumé solution per 1000 sq. ft. of paperboard, and assembling the impregnated board into a laminated board.

2. In a process for producing corrugated fiberboard, the steps comprising treating at least one side of a paperboard, which is at least .004 inch thick, with a sodium silicate solution having a specific gravity of from about 10 to 30° Bé. and an  $\text{SiO}_2:\text{Na}_2\text{O}$  weight ratio of from about 3.00 to 3.50, controlling the distribution of the silicate in the paperboard so that the ratio between the percentage of sodium silicate in the outside .002 inch and the next lower .002 inch is from about 1.2 to 3.0, such control being accomplished by varying the silicate solution concentration inversely with the amount of size and directly with the moisture content and porosity of the paperboard, the total amount of silicate solution applied being equivalent to from about 1 to 5 pounds of 40° Bé. solution per thousand square feet of paperboard, corrugating the impregnated paperboard, and assembling it into a corrugated board.

ERNEST R. BOLLER.

RAYMOND F. REMLER.